# EUROPEAN PATENT SPECIFICATION

(11) **EP 0 035 406 B1**
(45) Date of publication and mention of the grant of the patent: **08.08.1984**
(21) Application number: 81300881.0
(22) Date of filing: 03.03.1981
(51) Int. Cl.: D06M 11/04, C23C 17/02, H01B 1/10

(54) **Electrically conducting fibres and method of making same**
Elektrisch leitende Fasern und Verfahren zu ihrer Herstellung
Fibres électro-conductrices et procédé pour leur fabrication

(30) Priority: 05.03.1980 JP 28386/80; 15.07.1980 JP 97128/80
(43) Date of publication of application: 09.09.1981
(73) Proprietor: NIHON SANMO DYEING CO., LTD., Kyoto 612 (JP)
(72) Inventor: Tomibe, Shinji, Fushimi-ku Kyoto 612 (JP); Gomibuchi, Reizo, Uji-shi Kyoto 611 (JP); Takahashi, Kiyofumi, Yawata-shi Kyoto 614 (JP)
(74) Representative: Diamond, Bryan Clive

## Description

This invention relates to electrically conducting acrylic and modacrylic fibres and to methods of making them.

Numerous methods for imparting electrical conductivity to synthetic polymeric fibres are known. For example, one method for imparting electrical conductivity to polymeric fibres involves plating a metal onto the surface of the fibre. However, this method requires etching of the surface of the fibre prior to plating so as to obtain satisfactory adhesion, and then involves sensitising and activating the fibre prior to plating. In addition, the resulting electrically conducting fibre differs greatly from the starting fibre in softness, flexibility and smoothness.

In another prior art process, a metal is kneaded into a polymer. The polymer is then spun into a yarn. However, this process suffers from problems such as clogging of the nozzle with metallic particles during spinning. In addition, unless the metal content of the fibres is kept relatively low, the electrically conducting fibre obtained by this prior method has inferior mechanical properties compared to the starting fibre.

In a third known process, metallic powder is deposited in the pores of a polymeric fibre. This method usually requires an extremely porous fibre and intricate process steps.

U.S Patents 3,014,818 and 4,122,143 disclose the production of electrically conductive fibres by reducing a copper compound to metallic copper. In U.S. Patent 3,014,818, an electrically conductive fibrous material is produced by soaking the fibres, such as cotton or acrylic fibres, in a bath comprising a reducible salt of nickel, cobalt, copper or iron; the fibre is then subjected to a reducing treatment to obtain free metal particles which are dispersed through the interior of the fibre. Sodium borohydride and hydroxylamine are disclosed as satisfactory reducing agents. In U.S. Patent 4,122,143, cured products are obtained by reducing copper simultaneously with the curing of a resin; the method does not give electrical conductivity to an already existing fibre.

In the latter two known processes, electrical conductivity is obtained by the presence of metallic copper in the polymeric material. However, it is well-known that acrylic or modacrylic fibres have a strong affinity for monovalent copper ions; it is believed that this results from coordinate bonding between the cyano groups in the fibre and the monovalent copper ions. The adsorption of monovalent copper ions into acrylic or modacrylic fibres turns the fibres yellowish. However, as determined e.g. by measurements of electrical resistance, the fibres themselves do not possess any electrical conductivity.

Electrically conducting fibres having superior conductivity which is not lost in repeated washings are obtained without the need for special pretreatment of the fibres by means of this invention.

G.B. Specification No. 1,372,656 (and the corresponding U.S. Patent 3,940,533) discloses synthetic polymers which have a metal compound deposited on and/or within the fibres, by a process in which the fibre is treated with hydrogen sulfide or thioacetamide or thiourea as sulfur-containing compound, and then treating with an aqueous solution of a reactive metal salt, e.g. copper sulfate, chloride or acetate; the treated fibre is dried, e.g. at 60°C. The treated fibre is said to have good electrical conductivity and antistatic properties. The only synthetic polymers specifically described are polyamides, polyesters and polyamideimides.

According to the present invention, electrically conducting synthetic polymeric fibres have a copper sulfide adsorbed on the fibres, and the fibre is acrylic or modacrylic.

Suitable copper sulfides are cupric or cuprous sulfide or digenite.

Acrylic fibres are made from a synthetic linear polymer that consists of not less than 85% (by mass) of acrylonitrile units or acrylonitrile copolymers; modacrylic fibres contain not less than 35% of said units or copolymers. The term "fibre" or "acrylic fibre" is used hereinafter to refer to acrylic and modacrylic fibres.

The greater the quantity of copper ions present adsorbed by the fibre, the better the electrical conductivity of the product fibres. However, if the copper ion content is too high the physical properties, such as fibre strength and color, are affected. On the other hand, satisfactory electrical conductivity properties cannot be obtained at very low copper ion contents. The preferred amount of monovalent copper ions adsorbed by the fibre is from 1 to 30% by weight (expressed in terms of the weight of metallic copper) based upon the initial weight of the fibre.

In one embodiment of the process of the present invention for making these fibres, an acrylic fibre or modacrylic fibre is first heat-treated in a bath containing a divalent copper compound and a reducing agent so that the fibre adsorbs the monovalent copper ions; the fibre is then heat-treated with a sulfur-containing compound to convert the adsorbed monovalent copper ions into a copper sulfide. This is a two-step process.

No special pretreatment of the fibres is needed. The touch and other physical characteristics of the starting acrylic or modacrylic fibre is preserved in the process of the present invention; the electrically conductive fibres of the invention have superior electrical conductivity and washability and can be dyed by cationic dyes.

In the first stage of this process of the present invention, the fibres are heat-treated in a bath containing a compound providing divalent copper ion and a reducing agent, so that monovalent copper ions are adsorbed by the fibres. The bath can optionally contain, for adjusting the pH of the bath to preferably 1.5 to 2.0, an acid or an acid salt such as sulfuric acid, hydrochloric acid or a salt thereof.

Suitable copper compounds which provide, by reaction with the reducing agent, monovalent copper ions for adsorption on the fibres are cupric salts, such as cupric sulfate, chloride, nitrate or acetate and chelate compounds of copper. Suitable reducing agents for inclusion in the bath are metallic copper, hydroxylamine, ferrous sulfate, ammonium vanadate, sodium hyphosphite, glucose and furfural.

The bath temperature is preferably in the range from 90°C to 110°C so as to efficiently adsorb the monovalent copper ions and to maintain the strength of the fibres. At temperatures below 90°C, it takes many hours to complete adsorption. At temperatures over 110°C, the strength of the fibres drops.

In the first stage of this process of the present invention, the acrylic fibres having adsorbed monovalent copper ions become yellowish but do not possess any electrical conductivity. Electrical conductivity is imparted to the fibres in the second stage, wherein the fibres having adsorbed monovalent copper ions are preferably first thoroughly scoured or washed with water and the washed fibres are heat-treated in a liquid or gas which comprises a sulfur-containing compound which is capable of reacting with the adsorbed monovalent copper ions to produce a copper sulfide. The copper sulfide is adsorbed into the fibres, thereby imparting excellent electrical conductivity properties to the fibres. The weight percentage of the copper sulfide in the electrically conducting fibre expressed in terms of the weight of metallic copper is preferably also 1% to 30% based upon the initial weight of the fibre.

Suitable sulfur-containing compounds for converting the monovalent copper ions into adsorbed copper sulfide are sodium sulfide, sulfur dioxide, sodium hydrogen sulfite, sodium pyrosulfite, sulfurous acid, dithionous acid, sodium dithionite, sodium thiosulfate, thiourea dioxide, hydrogen sulfide, sodium formaldehyde sulphoxylate and zinc formaldehyde sulphoxylate and mixtures thereof. The liquid which contains the sulfur-containing compounds is generally water, and for adjusting the pH values to preferably 5.5 to 6 can include an acid or an acid salt such as sulfuric acid, sodium acetate or hydrochloric acid.

The heat-treatment temperature in the second stage of this process of the present invention is preferably more than 50°C. Heat-treatment temperatures below 50°C do result in the production of a copper sulfide and impart electrical conductivity to the fibres, but many hours are needed to accomplish this at these low temperatures. Suitably, the heat-treating in the second stage of the process of the present invention is at a temperature from 50°C to 105°C for about 1 hour and can be carried out in a gaseous sulfur-containing compound, such as sulfur dioxide.

In a second embodiment of the process of the invention an acrylic or modacrylic fibre is heat-treated in a bath containing (i) a divalent copper compound, (ii) a reducing agent capable of reducing said copper ions to monovalent ions, and (iii) a compound having the ability to release sulfur atoms and/or sulfur ions. This one-step process is simple to perform.

In this second method, as the compound (i) providing divalent copper ions, cupric compounds such as cupric sulfate, chloride, nitrate or acetate or a chelate of copper are used. The reducing agent (ii) can be metallic copper, ferrous sulfate, ammonium vanadate, sodium hypophosphite, hydroxylamine or its sulfate, furfural or glucose. The sulfur-releasing compound can be any of the sulfur containing compounds listed above for the first process; the sulphoxylates can be used in the form of sodium or zinc formaldehyde sulphoxylate or sulfur dioxide or hydrogen sulfide can be used by being bubbled into the bath. The sulfur-containing compound may also serve as at least part of the reducing agent. Further, in order to regulate the pH, acid or salt may be added, e.g. inorganic acid such as sulfuric or hydrochloric acid, organic acid such as citric acid or acetic acid or a combination of acid and salt such as citric acid and disodium hydrogen phosphate.

The treatment temperature used in this one-step method is normally 50°C to 120°C; a temperature higher than 120°C is liable to reduce the fibre strength, although the reaction will be quicker.

An electrically conducting fibre prepared by either process is washed thoroughly, e.g. with water, and then dried. Electrically conducting fibres obtained by the processes of the present invention were analyzed by X-ray diffraction techniques for the determination of the crystal structure of the adsorbed copper sulfide. It was thereby ascertained from the diffraction lines that the copper sulfide was adsorbed within the fibres in the form of digenite (empirical formula: C_{U}gSg), cuprous sulfide or cupric sulfide.

The respective interfacial distances in 10-¹⁶ metres of the copper sulfides are:-

In each process, the copper compound and/or reducing agent used can be a single compound or a suitable mixture of compounds.

Adsorption of the copper sulfide within the whole fibre results in a fibre which possesses excellent electrical conductivity and washability, and the touch and physical properties of the starting fibre is substantially preserved.

The electrically conducting fibres of the present invention can be dyed, e.g. with cationic dyes. (Electrically conducting fibres produced by the metal plating method cannot be dyed.) Suitably, the electrically conducting fibres of the present invention are dyed in an aqueous solution containing cationic dye at a temperature of about 100°C for about 30 minutes to 1 hour.

An electrically conducting fibre of the present invention can be used for many purposes. It can be used alone or in combination with other fibres to produce woven or knitted fabrics for electric blankets, electrically heated clothing and the like. Excellent control over the electrical properties of knitted or woven goods is obtained by combining in one textile the electrically conductive fibres of the present invention with other non-conductive fibres. For example, a small amount of the electrically conductive fibres of the present invention can be mingled into knitted or woven goods in the form of filament fibres. Also, spun yarns can be produced from mixtures of the electrically conductive fibres of the present invention with other natural or synthetic fibres which are both in the form of staple fibres.

The invention is illustrated but not limited by the following examples in which all percentages and ratios are by weight. The No. 31 mesh has 12 openings per square of side 1 inch (2.54 cm) long. The washing test involves washing the sample in a rotating drum in soapy water for 30 minutes at 50°C.

### Example 1

An acrylic fibre of 2 deniers (0.22 tex) yarn and 51 millimetres in length of cut, marketed as Cashmilon, type FWBR, by Asahi Chemical Industry Co., Ltd. of Japan, was heat-treated in an aqueous bath containing 30 wt.% of cupric sulfate, 4% of sulfuric acid and 80% of copper net (No. 31, of a 12-mesh) in relation to the weight of the fibre in the bath. The ratio of the fibres to water containing the chemicals was 1:15. The heat-treatment was at a temperature of 95°C for 60 minutes. Subsequently, the fibres were thoroughly washed in water.

The washed fibres were again heat-treated in an aqueous solution containing 10 grams of sodium formaldehyde sulphoxylate (Rongalite C, and 1 millilitre of sulfuric acid in relation to 1 litre of water, at a temperature of 80°C for 60 minutes. The electrically conducting fibre was dried after being washed in water for a second time. It had an olive-grey colour and contained 12.3% of copper sulfide in relation to the weight of the starting fibre. Its electrical resistivity was 0.085 ohm.centimetre. The crystal structure of this electrically conducting fibre was analyzed by X-ray diffraction; the line of diffraction (interfacial distance 10-¹⁰ m: 1.97, 3.21, 2.79) was of digenite (empirical formula: cu₉^{s}_{'}).

When this electrically conducting fibre was subjected ten times to the repeated washing test according to Japanese Industrial Standard L-1045, A-2, its electrical resistivity was 0.090 ohm.centimetre and its washability was excellent.

This electrically conducting fibre was treated in an aqueous solution containing 2% of Sumiacryl Brilliant Red N-4G (cationic dye, made by Sumitomo Chemical Industry Co., Ltd., Japan) in relation to the fibre weight at a temperature of 100°C for 30 minutes. It was excellently dyed a dark-red colour without deterioration of its conductivity.

### Example 2

Example 1 was repeated except that zinc formaldehyde sulphoxylate was used in place of sodium formaldehyde sulphoxylate. There was likewise obtained an electrically conducting fibre of the same nature as the fibre obtained in Example 1.

### Example 3

A modacrylic fibre of 2 deniers (0.22 tex) yarn and 51 millimetres in length of cut, marketed as Kanekalon S made by Kane- gafuchi Chemical Co., Ltd., Japan, was heat-treated in a bath containing 30% of cupric sulfate and 15% of hydroxylamine sulfate in relation to the weight of fibre in the bath. The ratio of the fibres to the water containing the chemicals was 1:15. The heat-treatment was at a temperature of 100°C for 90 minutes. The fibres were then thoroughly washed in water.

The washed fibres were again heat-treated in an aqueous solution containing 10 grams of dithionous acid and 2 grams of sodium acetate per litre of water, at a temperature of 90°C for 60 minutes. The electrically conducting fibre obtained after being thoroughly washed in water and dried had an olive-grey colour and contained 10.8% of copper sulfide in relation to the weight of the starting fibre. Its electrical resistivity was 0.86 ohm-centimetre.

When this electrically conducting fibre was subjected ten times to the repeated washing test as in Example 1, deterioration of its conductivity was scarcely perceived. Further, this electrically conducting fibre was treated in an aqueous solution containing 2% of Diacryl Brilliant Blue H_{z}R-N (cationic dye, made by Mitsubishi Chemical Industry Co., Ltd., Japan) in relation to the fibre weight at a temperature of 100°C for 60 minutes. The electrically conducting fibre was excellently dyed a dark-blue colour.

### Examples 4-7

The procedure of Example 3 was repeated except that instead of dithionous acid, either sodium dithionite, sodium thiosulfate, sodium hydrogen sulfite or sodium pyrosulfite was used. In each case, there was obtained an electrically conducting fibre of the same nature as the fibre obtained in Example 3.

### Example 8

An acrylic fibre of 3 deniers (0.33 tex) yarn and 102 millimetres in length of cut, marketed as Toraylon type T-106, made by Toray Industry, Inc., Japan, was heat-treated in a bath containing 40% of cupric chloride and 20% of hydroxylamine sulfate in relation to the weight of fibre in the bath. The ratio of fibres to water containing the chemicals was 1:15. The heat-treatment was at a temperature of 100°C for 60 minutes. Subsequently, the fibres were thoroughly washed in water.

The washed fibres were again heat-treated in an aqueous solution containing 15 grams of sodium sulfide and 4 millilitres of sulfuric acid per litre of water, at a temperature of 90°C for 60 minutes. The electrically conducting fibre obtained after being thoroughly washed in water and dried had an olive-grey color and contained 15.1% by weight copper sulfide in relation to the weight of the starting fibre. Its electrical resistivity was 0.060 ohm.centimetre.

When this electrically conducting fibre was subjected to the repeated washing test as in Example 1, deterioration of its conductivity was negligible.

Further, this electrically conducting fibre was treated in an aqueous solution containing 4% of Diacryl Navy Blue RL-N (cationic dye, made by Mitsubishi Chemical Industry Co., Ltd., Japan) in relation to the fibre weight, at a temperature of 100°C for 60 minutes. An electrically conducting fibre dyed well in a dark-blue colour was obtained.

### Example 9

An acrylic fibre of 2 deniers (0.22 tex) yarn and 51 millimetres in length of cut, marketed as Cashmilon by Asahi Chemical Industry Co., Ltd., Japan, which had been treated to adsorb monovalent copper ions through the same treatment as in Example 1, was put into a closed receptacle having a gas inlet. Sulfur dioxide was fed into the receptacle until the pressure in the interior thereon reached 0.5 kg/cm² gauge pressure. Then, saturated water vapour at 105°C was fed into the receptacle until the pressure within the receptacle reached 1.0 kg/cm² gauge pressure. After the receptacle had been shut tightly, the fibres reacted therein with the sulfur dioxide. They were taken out after cooling, washed thoroughly in water and dried. The electrically conducting fibre thus obtained had an olive-grey colour. Its electrical resistivity was 0.50 ohm.centimetre.

The electrically conducting fibre was tested for washability and dyeability by cationic dyestuffs. The results were as good as in the case of Examples 1 to 8.

### Example 10

Example 9 was repeated except that hydrogen sulfide was used instead of sulfur dioxide. An electrically conducting fibre of the same nature as the fibre obtained in Example 9 was obtained.

### Example 11

An acrylic fibre of 2 deniers (0.22 tex) yarn and 51 mm in length of cut, Casmilon type FWBR, made by Asahi Chemical Industry Co., Ltd., was first thoroughly scoured, and then heat-treated in a bath containing 30 wt.% of cupric sulfate, 15% of sodium thiosulfate and 15% of sodium hydrogen sulfite in relation to the weight of the fibre in the bath. The ratio of the fibres to the water containing the chemicals was 1:15. The treatment was for 60 minutes at the temperature of 75°C, to which temperature the bath had been raised over 30 minutes from the room temperature. The fibres were then washed in water and dried.

The conductive fibre thus obtained has an olive green color, a copper sulfide content of 14.2% and an electrical resistivity of 0.036 ohm.centimetre. X-ray diffraction analysis showed it to contain cupric or cuprous sulfide or digenite.

After the repeated washing test ten time as in Example 1, its resistivity had increased only slightly to 0.043 ohm.cm.

This electrically conducting Cashmilon fibre was also dyed as in Example 1.

### Example 12

An acrylic fibre of 3 deniers (0.33 tex) yarn and 51 mm in length of cut, marketed as Kane- boacryl type BR VO-1, by Kanebo Synthetic Fibre Co., Ltd., Japan, was heat-treated as in Example 11 but in a bath containing 20% of cupric sulfate, 10% of sodium pyrosulfite and 10% of hydroxylamine sulfate and for 120 minutes at 50°C (reached after 15 minutes).

The conductive fibre obtained was olive green, contained 13.8% copper sulfide, had a resistivity of 0.058 ohm.cm, and showed digenite diffraction lines.

After the repeated washing test its resistivity was 0.063 ohm.cm and its washability was good.

The electrically conducting fibre was treated in an aqueous solution of Diacryl Navy Blue RL-N (cationic dye, made by Mitsubishi Chemical Industry Co., Ltd., Japan), and was dyed brilliantly navy blue without lowering the electric conductivity.

### Example 13

A modacrylic fibre as used in Example 3 was treated as in Example 11 but in a bath containing 20% of cupric sulfate, 80% of copper net (No. 31, of a 12 mesh), 10% of sodium thiosulfate and 5% of sulfuric acid for 60 minutes at 100°C (reached after 45 minutes).

The conductive fibre obtained was olive green, contained 9.2% copper sulfide, had a resistivity of 1.3 ohm.cm and showed digenite diffraction lines.

After the repeated washing test, its resistivity was 1.4 ohm.cm and its washability was good.

When this electrically conducting fibre was treated in an aqueous solution of Diacryl Brilliant Blue H₂R-N (cationic dye, made by Mitsubishi Chemical Industry Co., Ltd., Japan), it was dyed brilliantly dark blue, without lowering the electric conductivity.

## Claims

1. An electrically conducting synthetic polymeric fibre having copper sulfide adsorbed on the fibre, characterised in that the fibre is an acrylic or modacrylic fibre.

2. An electrically conducting fibre as claimed in Claim 1, wherein the amount of copper sulfide, expressed as metallic copper, is 1% to 30% of the weight of the starting fibre.

3. An electrically conducting fibre as claimed in Claim 1 or 2, wherein said copper sulfide is digenite.

4. An electrically conducting fibre as claimed in Claim 1 or 2, wherein said copper sulfide is cupric sulfide or cuprous sulfide.

5. An electrically conducting fibre as claimed in Claim 1, 2 or 3, which has been dyed with a cationic dye.

6. A method of making an electrically conducting fibre as claimed in Claim 1, 2, 3 or 4, by treating the fibre with a source of copper ions and a sulfur-containing compound, characterised in that it comprises subjecting an acrylic or modacrylic fibre to a first heat-treatment in a bath containing a cupric compound and a reducing agent so as to adsorb monovalent copper ions into the fibre, and subjecting the fibre to a second heat-treatment in the presence of a sulfur-containing compound to convert said adsorbed monovalent copper ions to a copper sulfide.

7. A method as claimed in Claim 6, wherein said fibre is washed between the first and second heat-treatments.

8. A method as claimed in Claim 6 or 7, wherein said first heat-treatment is at a temperature of from 90°C to 110°C.

9. A method as claimed in any of Claims 6, 7 or 8, wherein said second heat-treatment is at a temperature of from 50°C to 105°C.

10. A method as claimed in Claim 6, 7, 8 or 9, wherein said second heat-treatment is conducted in a gaseous sulfur-containing compound.

11. A method of making an electrically conducting fibre as claimed in Claim 1, 2, 3 or 4, by treating the fibre with a source of copper ions and a sulfur-containing compound, characterised in that it comprises subjecting an acrylic or modacrylic fibre to heat-treatment in a bath which contains a cupric compound, a reducing agent which is capable of reducing copper ions to monovalent ions, and a sulfur-containing compound to convert said monovalent copper ions to a copper sulfide.

12. A method as claimed in Claim 11, wherein said treatment is at a temperature of 50°C to 120°C.

13. A method as claimed in Claim 11 or 12 wherein said sulfur-containing compound also serves as at least part of the reducing agent.

14. A method as claimed in any of Claims 6 to 13, wherein said cupric compound is cupric sulfate, cupric chloride, cupric nitrate, cupric acetate or a chelate of copper.

15. A method as claimed in any of Claims 6 to 14, wherein said reducing agent is metallic copper, ferrous sulfate, ammonium vanadate, sodium hypophosphite, hydroxylamine or its sulfate, furfural or glucose.

16. A method as claimed in any of Claims 6 to 15, wherein said sulfur-containing compound is selected from sodium sulfide, sulfur dioxide, sodium formaldehyde sulphoxylate, zinc formaldehyde sulphoxylate, sodium pyrosulfite, sulfurous acid, dithionous acid, sodium dithionite, sodium thiosulfate, thiourea dioxide, hydrogen sulfide and sodium hydrogen sulfite.

17. A method as claimed in any of Claims 6 to 16, wherein the treated fibre is then dyed with a cationic dye.

## Patentansprüche

1. Elektrisch leitende synthetische polymere Fasern mit von der Faser adsorbiertem Kupfersulfid, dadurch gekennzeichnet, daß die Faser eine Acryl- oder Modacrylfaser ist.

2. Elektrisch leitende Faser nach Anspruch 1, dadurch gekennzeichnet, daß der Anteil an Kupfersulfid, ausgedrückt in metallischem Kupfer, 1 bis 30% des Gewichts der Ausgangsfaser beträgt.

3. Elektrisch leitende Faser nach Anspruch 1 oder 2, dadurch gekennzeichnet, daß das Kupfersulfid aus Digenit besteht.

4. Elektrisch leitende Faser nach Anspruch 1 oder 2, dadurch gekennzeichnet, daß das Kupfersulfid aus Kupfer(11)-Sulfid oder Kupfer(1)-Sulfid besteht.

5. Elektrisch leitende Faser nach einem der Ansprüche 1 bis 3, dadurch gekennzeichnet, daß sie mit einem kathionischen Farbstoff eingefärbt ist.

6. Verfahren zum Herstellen elektrisch leitender Fasern nach den Ansprüche 1 bis 4 durch Behandlung der Faser mit einem die Kupferionen enthaltenden Medium und einer Schwefel enthaltenden Verbindung, dadurch gekennzeichnet, daß eine Acryl- oder Modacryl-Faser zunächst einer ersten Wärmebehandlung in einem die Kupferverbindung und ein Reduktionsmittel enthaltenden Bad zur Absorption des einwertigen Kupferions durch die Faser und die Faser anschließend einer zweiten Wärmebehandlung in Gegenwart einer Schwefel enthaltenden Verbindung unterzogen wird, um das adsorbierte einwertige Kupferion in ein Kupfersulfid umzuwandeln.

7. Verfahren nach Anspruch 6, dadurch gekennzeichnet, daß die Faser zwischen der ersten und der zweiten Wärmebehandlung ausgewaschen wird.

8. Verfahren nach Anspruch 6 oder 7, dadurch gekennzeichnet, daß die erste Wärmebehandlung bei einer Temperatur von 90 bis 110°C durchgeführt wird.

9. Verfahren nach einem der Ansprüche 6 bis 8, dadurch gekennzeichnet, daß die zweite Wärmebehandlung bei einer Temperatur von 50 bis 105°C durchgeführt wird.

10. Verfahren nach den Ansprüchen 6 bis 9, dadurch gekennzeichnet, daß die zweite Wärmebehandlung in einer gasförmigen Schwefel enthaltenden Verbindung durchgeführt wird.

11. Verfahren zum Herstellen elektrisch leitender Fasern nach den Ansprüchen 1 bis 4 durch Behandlung der Faser mit einem Kupferionen enthaltenden Medium und einer Schwefel enthaltenden Verbindung, dadurch gekennzeichnet, daß eine Acryl- oder Modacrylfaser einer Wärmebehandlung in einem Bad, das eine Kupferverbindung, ein die Kupferionen zu einwertigen Ionen reduzierendes Reduktionsmittel und eine Schwefel enthaltende Verbindung zur Umwandlung des einwertigen Kupferions in ein Kupfersulfid enthält, unterzogen wird.

12. Verfahren nach Anspruch 11, dadurch gekennzeichnet, daß die Wärmebehandlung bei einer Temperatur von 50 bis 120°C durchgeführt wird.

13. Verfahren nach Anspruch 11 oder 12, dadurch gekennzeichnet, daß die Schwefel enthaltende Verbindung zugleich zumindest ein Teil des Reduktionsmittels bildet.

14. Verfahren nach einem der Ansprüche 6 bis 13, dadurch gekennzeichnet, daß die Kupfer(11)-Verbindung Kupfersulfat, Kupferchlorid, Kupfernitrat, Kupferacetat oder ein Kupferchelat ist.

15. Verfahren nach einem der Ansprüche 6 bis 14, dadurch gekennzeichnet, daß das Reduktionsmittel metallisches Kupfer, Ferrosulfat, Ammoniumvanadat, Natriumhypophosphit, Hydroxylamin oder deren Sulfate, Furfural oder Glucose ist.

16. Verfahren nach einem der Ansprüche 6 bis 15, dadurch gekennzeichnet, daß die Schwefel enthaltende Verbindung aus Natriumsulfid, Schwefeldioxid, Natriumformaldehyd, Sulfoxylat, Zinkformaldehyd-Sulfoxylat, Natriumpyrosulfit, Schweflige Säure, Dithionsäure, Natriumdithionid, Natriumthiosulfat, Thioharnstoffdioxid, Hydrogensulfid oder Natrium-Hydrogensulfit ausgewählt ist.

17. Verfahren nach einem der Ansprüche 6 bis 16, dadurch gekennzeichnet, daß die behandelte Faser anschließend mit einem kathionischen Farbstoff eingefärbt wird.

## Revendications

1. Fibre polymère synthétique électro-conductrice sur laquelle est adsorbé du sulfure de cuivre, caractérisée en ce que la fibre est une fibre acrylique ou une fibre modacrylique.

2. Fibre électro-conductrice selon la revendication 1, dans laquelle la quantité de sulfure de cuivre, exprimée en cuivre métallique, est 1 à 30% du poids de la fibre de départ.

3. Fibre électro-conductrice selon la revendication 1 ou 2, dans laquelle le sulfure de cuivre est de la digénite.

4. Fibre électro-conductrice selon la revendication 1 ou 2, dans laquelle le sulfure de cuivre est un sulfure cuivrique ou un sulfure cuivreux.

5. Fibre électro-conductrice selon la revendication 1, 2 ou 3, qui a été teinte avec un pigment cationique.

6. Procédé de préparation d'une fibre électro-conductrice selon la revendication 1, 2, 3 ou 4, en traitant la fibre avec une source d'ions de cuivre et un composé contenant du soufre, caractérisé en ce qu'on soumet une fibre acrylique ou modacrylique à un premier traitement à chaud dans un bain contenant un composé cuivrique et un agent réducteur de façon à adsorber des ions de cuivre monovalent dans la fibre, et on soumet la fibre à un deuxième traitement thermique en présence d'un composé contenant du soufre pour transformer les ions de cuivre monovalent adsorbés en sulfure de cuivre.

7. Procédé selon la revendication 6, dans lequel la fibre est lavée entre le premier traitement à chaud et le deuxième traitement à chaud.

8. Procédé selon la revendication 6 ou la revendication 7, dans lequel le premier traitement à chaud s'effectue à une température comprise entre 90 et 110°C.

9. Procédé selon l'une quelconque des revendications 6, 7 ou 8, dans lequel le deuxième traitement à chaud s'effectue à une température comprise entre 50 et 105°C.

10. Procédé selon la revendication 6, 7, 8 ou 9, dans lequel le deuxième traitement à chaud est effectué dans un composé gazeux contenant du soufre.

11. Procédé de préparation d'une fibre électro-conductrice selon la revendication 1, 2, 3 ou 4, en traitant la fibre avec une source d'ions de cuivre et un composé contenant du soufre, caractérisé en ce qu'on soumet une fibre acrylique ou modacrylique à un traitement à chaud dans un bain qui contient un composé cuivrique, un agent réducteur capable de réduire les ions de cuivre en ions monovalents, et un composé contenant du soufre pour transformer les ions de cuivre monovalent en sulfure de cuivre.

12. Procédé selon la revendication 11, dans lequel le traitement s'effectue à une température comprise entre 50° et 120°C.

13. Procédé selon la revendication 11 ou 12, dans lequel le composé contenant du soufre sert également au moins partiellement d'agent réducteur.

14. Procédé selon l'une des revendications 6 à 13, dans lequel le composé cuivrique est du sulfate cuivrique, du chlorure cuivrique, du nitrate cuivrique, de l'acétate cuivrique ou un chélate de cuivre.

15. Procédé selon l'une quelconque des revendications 6 à 14, dans lequel l'agent réducteur est du cuivre métallique, du sulfate ferreux, du vanadate d'ammonium, de l'hypophosphite de sodium, de l'hydroxylamine ou son sulfate, du furfural ou du glucose.

16. Procédé selon l'une quelconque des revendications 6 à 15, dans lequel le composé contenant du soufre est choisi parmi le sulfure de sodium, le bioxyde de soufre, le sulfoxylate- formaldéhyde de sodium, le sulfoxylate- formaldéhyde de zinc, le pyrosulfite de sodium, l'acide sulfureux, l'acide hydrosulfureux, l'hydro- sulfite de sodium, le thiosulfate de sodium, le bioxyde de thiourée, le sulfure d'hydrogène et l'hydrogénosulfite de sodium.

17. Procédé selon l'une quelconque des revendications 6 à 16, dans lequel la fibre traitée est ensuite teinte avec un pigment cationique.
